

Nov. 21, 1950

A. H. WARTH

2,530,413

CONTAINER

Filed Oct. 29, 1945

*Fig. 1.*



*Fig. 2.*



*Fig. 3.*



*Fig. 4.*



Inventor:

*Albin H. Warth,  
By Cushman, Darby & Cushman*

Attorneys.

## UNITED STATES PATENT OFFICE

2,530,413

## CONTAINER

Albin H. Warth, Baltimore, Md., assignor to  
 Crown Cork & Seal Company, Inc., Baltimore,  
 Md., a corporation of New York

Application October 29, 1945, Serial No. 625,246

3 Claims. (Cl. 220—64)

**1**  
 This invention relates to containers particularly those for packaging foods and beverages, in which a metallic surface comes into contact with the container contents. In addition, the invention is concerned with new alloys, metal coated with these new alloys and containers comprising such alloys.

Considerable difficulty has been encountered in the production of completely satisfactory containers and packages for food and beverages, particularly those of a high acidic content such as citrus fruit juices and the like. As is fully described in my co-pending application, Serial No. 439,292, filed April 16, 1942, and now abandoned, ordinary tin plate is not an entirely satisfactory material from which to fabricate containers for fruit juices because of the loss of aroma, flavor and discoloration of the contents upon ageing in the container. On the other hand, the use of containers in which a metallic surface is exposed to the container contents is advantageous in the packaging of acidic foods and beverages if the metal surface exposed evolves a minute amount of nascent hydrogen during storage of the packaged product. This advantage resides in the ability of the nascent hydrogen to maintain the packaged material free from oxidation and other resulting changes in flavor and discoloration which accompany the oxidation processes. In this respect, containers having a metal surface exposed to the packaged product are superior to containers in which only non-metallic surfaces are exposed to the acidic packaged material, e. g., containers of glass or metal containers lined with enamel or organic resinous coatings.

Ordinarily, tin plate is the most common material used in the preparation of food or beverage containers made wholly or partially of metal. However, this material is not entirely satisfactory for use in the packaging of acidic foods and beverages because of excessive chemical attack upon the tin plate by the container contents. Various modifications of tin plate have been attempted in order to overcome this disability, e. g., the use of an alloy of tin with minor amounts of silver, as in my above mentioned patent application, for the production of coated sheet metal to be employed in the production of the containers. However, even these improvements over the common tin plate have not resulted in the elimination of all of the deficiencies associated with containers made from such coated metals. Thus, the silver modified tin plate is subject to tarnishing and its corrosion resistance is not as high as is desirable.

**2**  
 A principal object of this invention is to overcome all of the deficiencies of the subject containers as described above. A further object is the provision of containers having at least a portion of the surface exposed to the container contents made from metal, said metal surface being highly resistant to corrosion and oxidation.

A further object is the provision of plated sheet metal having a plating which is tougher than tin and containers fabricated from such plated metal. Another object is the provision of plated metal from which food and beverage containers may be produced which exhibit extremely good soldering characteristics. Further objects and the entire scope of applicability of the present invention will become apparent from the detailed description given hereinafter.

These objects are accomplished according to the present invention by the preparation of an alloy comprising tin, silver and indium, the plating of a base metal sheet with this alloy and the fabrication of containers for foods and beverages from such alloys or coated metal sheets in which any of the metal surfaces of the container exposed to the packaged material is made of the alloy.

The success of this invention resides primarily in the discovery that an alloy composed of a major proportion of tin and a minor proportion of silver and indium provides a sufficient amount of nascent hydrogen upon contact with acidic foods or beverages to keep the true flavor of container contents during storage while exhibiting an extremely good degree of chemical and corrosion resistance and attractive appearance without tarnishing or undergoing oxidation. The manner in which this discovery is utilized may be stated as follows:

Sheet metal, such as black iron or steel of a gauge or thickness adapted to permit fabrication of containers from the metal is coated with an alloy comprising tin, silver and indium, such as an alloy of 93 to 100 parts of tin, 0.1 to 3.5 parts of silver and 0.03 to 3.5 parts of indium. The coating of the metal sheet may be accomplished by a hot dipping procedure, i. e., by dipping the sheet in the molten metal alloy; by an electrolytic process, i. e., plating the sheet metal in an electrolytic bath of an acid or alkaline nature containing silver, tin and indium in the proper proportions to yield the desired coating; or by a vaporlytic process, i. e., by vaporizing the alloy in a vacuum chamber and condensing the vapor upon the sheet metal plate. Moreover, a container may be fabricated from the uncoated base

metal plate and then coated with the alloy by any of the methods indicated above.

The alloy need not be used for making the entire surface of the container, but is also satisfactory for use in the preparation of container closures having an overall or center-spot facing coated or made from the alloy. Thus, a tin metal foil may be coated with the alloy for production of container closures facings or thin foil may be prepared from the alloy. Such foil may be made in substantially the same manner as is used to prepare tin metal foil, e. g., rolling. The tin-silver-indium foil can be also mounted on paper material by means of a thermoplastic adhesive, preferably by coating the paper and then by means of heat and pressure wedged to the metal foil. The advantage is that a somewhat thinner foil can be successfully used, namely, .001" foil or a trifle less, which can be mounted on a paper having .002" thickness or a trifle less. When using silver-tin-indium foil without paper mounting, a thickness of at least .00015" is used, due to rupture of thinner foils in the mechanical assembly of the spot or overall facing on the disc or solid liner of the crown. Ordinary tin foil is not generally used with a thickness of less than .002" for Spot Crowns, but the silver-tin-indium foil is stronger and somewhat easier to handle and a lesser thickness may be satisfactory, but usually the tin-silver-indium alloy foil is of a thickness in the neighborhood of about .002".

For the purpose of illustrating the invention I have shown in the accompanying drawing a container and a cap coated with the silver-tin-indium alloy. It is to be understood that various types of containers and caps as well as other articles employed for packaging foods and beverages may be similarly lined or provided with exterior coating as described herein.

Referring to the drawings:

Figure 1 is an elevation partly in section of a can such as a sanitary type can having a lining of the tin-silver-indium alloy.

Figure 2 is a sectional view of a can-end for use with the can of Figure 1, similarly lined.

Figure 3 is a sectional view of a crown cap having its exterior surface coated with my improved alloy, and

Figure 4 is a sectional view of a crown cap having a cushion liner coated with a film of the tin-silver-indium alloy on its exposed surface which may be in the form of an overall or center-spot facing.

The can 10 shown in Figure 1 is provided with a seam 11, which may be sealed with either ordinary solder, with tin-silver-indium solder or similar materials. Alloys of tin with 3½ to 10 percent silver may be used for solders that require greater corrosion resistance than lead-tin solders, or where it is desirable to eliminate the toxic lead. The alloy lining is indicated at 13 and is coextensive with the interior wall of the container. The alloy may also be coated upon the exterior of the can to be coextensive therewith, and I have found that it is highly receptive of the usual can decorations and likewise imparts a bright finish.

The end shown in Figure 2 is the customary can end for sealing a standard sanitary can, as shown in Figure 1, and has its inner or exposed surface coated with the alloy lining 13. The exterior surface of the end may also be similarly coated.

The cap 14 shown in Figure 3 has a cushion liner 17 and has its exterior surface provided with

an alloy coating of tin-silver-indium alloy in accordance with this invention. This coating, as just stated, will impart a bright finish and will readily receive the lithograph or other printing decoration. The standard sanitary can shown in Figure 1 is made of metal plate such as black iron or steel, previously coated with the improved tin-silver-indium alloy and then folded or bent in the usual manner into a can body by the customary body making machinery and the seam 11 sealed in the regular way. The cap is likewise made from coated plate, but instead of being bent to form, is stamped or drawn from the coated sheet.

Referring to Figure 4, the crown cap is provided with a cushion liner 15 of paper board, cardboard, or other solid material and has secured to its exposed face a film 16 of the tin-silver-indium alloy as described herein, e. g., tin-silver-indium alloy foil and constituting an overall or center-spot facing.

A more complete comprehension of the present invention may be had from the following illustrative example, in which all parts are by weight:

#### Example

This example illustrates the preparation of container of the sanitary can type from sheet metal prepared by hot dipping process.

A hot dipping bath is prepared by melting together 20 parts of silver, 7 parts of indium and 970 parts of tin containing 3 parts of impurities. The melting point of this resulting alloy is about 230° C. and bright finish black plate is readily coated with the alloy using an ordinary dipping process, since the alloy has excellent flowing qualities and readily wets the sheet metal base.

The coated sheet metal is fabricated into a container of the sanitary can type, such as that illustrated in Figure 1, by the general can making procedure. It is found that this metal is particularly useful for this purpose in view of the ease with which the can seams may be soldered.

Orange juice is packaged in the resulting container. After storage for a considerable time, the orange juice is found to possess substantially the same color, aroma and flavor which it had before packaging. Moreover, all of the surfaces of the container exposed to the atmosphere during storage retain a bright, untarnished appearance and the inner can surfaces show substantially no signs of corrosion.

In another case, sheet metal was coated with ordinary tin and this tin plate was used to prepare containers and package orange juice. The orange juice stored in this latter container for the same period of time as the former, was found upon inspection to possess a distinctly changed aroma and flavor as compared to the orange juice originally packaged.

In still another case a container was made from sheet metal coated with an alloy of 97 parts of tin and 3 parts of silver. The chemical resistance of this last container to the action of the packaged orange juice was superior to that of the container made from plain tin plate, but was inferior to the container made from metal coated with the tin silver and indium alloy. On the other hand, the tin-silver coated container tarnished considerably during storage.

It is apparent from the description given above that the composition of the alloy coating of this invention may be varied. The exact composition of the alloy will depend in part upon the particular type of container into which the alloy is to

be fabricated and upon the type of metal to be packaged in the container. The most desirable alloys appear to be those in which the proportion of tin to silver is between 1000 to 1 and 27 to 1 and in which the proportion of silver to indium in the alloy is between 1 to 1 and 7 to 1. Particularly useful alloys are those comprising 93 to 100 parts of tin, 0.1 to 3.5 parts of silver and 0.03 to 3.5 parts of indium. An especially useful alloy is composed of 97 parts of tin, 2 parts of silver and 0.7 part of indium.

This invention provides new and useful alloys which may be employed for applications where high degrees of chemical resistance coupled with high degrees of toughness are required. Although these alloys are generally useful for these purposes, they are particularly applicable to the production of containers and container closures for packaging foods and beverages, particularly those of an acidic nature.

I claim:

1. A sheet metal container having a coating on its wall of an alloy composed of 93 to 100 parts of tin, 0.1 to 3.5 parts of silver and 0.03 to 3.5 parts of indium, except for incidental impurities.

2. A container closure having on its interior a coating composed of 93 to 100 parts of tin, 0.1 to 3.5 parts of silver and 0.03 to 3.5 parts of indium, except for incidental impurities.

3. An alloy composed of 93 to 100 parts of tin, 30

0.1 to 3.5 parts of silver and 0.03 to 3.5 parts of indium, except for incidental impurities.

ALBIN H. WARTH.

#### REFERENCES CITED

The following references are of record in the file of this patent:

#### UNITED STATES PATENTS

|    | Number    | Name            | Date          |
|----|-----------|-----------------|---------------|
| 10 | 135,028   | Zimmer          | Jan. 21, 1873 |
|    | 250,326   | DeVilliers      | Nov. 29, 1881 |
|    | 1,437,641 | Ferriere et al. | Dec. 5, 1922  |
|    | 1,626,038 | Ireland         | Apr. 26, 1927 |
| 15 | 1,632,309 | Nitardy         | June 14, 1927 |
|    | 1,958,765 | Perkins         | May 15, 1934  |
|    | 2,151,032 | Scheller        | Mar. 21, 1939 |
|    | 2,157,933 | Hensel et al.   | May 19, 1939  |
|    | 2,241,789 | Queneau et al.  | May 13, 1941  |
| 20 | 2,364,713 | Hensel          | Dec. 12, 1944 |
|    | 2,373,352 | Smart           | Apr. 10, 1945 |
|    | 2,393,905 | Hensel          | Jan. 29, 1946 |

#### FOREIGN PATENTS

|    | Number  | Country       | Date          |
|----|---------|---------------|---------------|
| 25 | 565,072 | Great Britain | Oct. 25, 1944 |

#### OTHER REFERENCES

Metal Finishing, vol 40, 1942, pages 13-17.  
Product Engineering, Oct. 1943, pages 630-632.